

## UNITED STATES PATENT OFFICE

CAMILLE DREYFUS, OF NEW YORK, N. Y., AND WILLIAM WHITEHEAD, OF CUMBERLAND, MARYLAND, ASSIGNEES TO CELANESE CORPORATION OF AMERICA, A CORPORATION OF DELAWARE

## TEXTILE PROCESS AND PRODUCT

No Drawing.

Application filed February 10, 1930. Serial No. 427,418.

This invention relates to the rendering of yarns more amenable to textile operations, and relates more particularly to the treatment of yarn made of filaments of substantially continuous lengths to present them in a form wherein they may be knitted more satisfactorily.

An object of our invention is to so treat the surface of yarns or filaments that the same may be more easily handled in subsequent textile operations. A further object of our invention is to so treat yarns that the same may be employed for making knitted or other fabrics having a smoother and more uniform appearance than has heretofore been possible. Other objects of our invention will appear from the following detailed description.

In the knitting of yarns, particularly yarns of continuous filamentary structure, and especially in the circular knitting of fabric or hose in accordance with prior methods, often the stitches and loops do not have exactly similar shapes. The variation from the normal or desired shape is known as "stitch distortion", where the stitches do not form a suitable straight line along the rib of the fabric, or as "pin-holes", where the stitches are so formed that there are small holes of greater size than the normal spaces between or in the stitches so formed. We have come to the conclusion that this is probably due to lack of uniformity of the coefficient of friction between the filaments of the yarn and also between the yarn and the needles or other working parts of the knitting machine controlling the tension of the yarn and the shape of the stitch.

We have found that if the surfaces of the yarns or filaments are roughened in any suitable manner, the same can be knitted into more satisfactory fabrics, and may also be wound into more satisfactory packages which will stand more severe handling with less danger of slipping and collapsing.

In accordance with our invention, we render yarns, particularly yarns made of continuous filaments, more suitable for textile operations by applying thereto a material that tends to roughen or increase the coefficient of friction of the yarns or filaments.

The yarns to be treated are preferably made of filaments of substantially continuous lengths. Thus the yarn may be made of filaments made of organic derivatives of cellulose, of reconstituted cellulose or of natural silk. A composite yarn made of filaments of two or more kinds may be employed. The organic derivative of cellulose may be an organic ester of cellulose or cellulose ether.

Examples of organic esters of cellulose are cellulose acetate, cellulose formate, cellulose propionate, and cellulose butyrate, while examples of cellulose ethers are ethyl cellulose, methyl cellulose and benzyl cellulose.

As to materials to be applied to the yarn to increase the coefficient of friction, any suitable ones may be used. They may be pigments, preferably in finely divided form, such as barium sulphate, barium carbonate, barium phosphate, calcium sulphate, calcium carbonate, titanium dioxide, talc, zinc oxide, etc. However other solid materials such as starch and the like may be employed. The material may be applied to the yarn by running the yarn through a mass of the finely divided material while in the dry form, while the yarn is either dry or wetted with a liquid or solvent.

Preferably however, the pigment or other solid material is ground or mixed with liquids, oils or finishes, and more preferably with the finishing or lubricating material ordinarily applied to such yarn prior to the textile operation. However the use as a dispersing medium for the pigment of a liquid which readily evaporates, such as water or a volatile organic liquid like alcohol, is not excluded. Moreover the application to the yarn of the oils, finishes and pigments in separate operations is not excluded.

It is preferable to grind the pigments or insoluble material to a fine and uniform size, which may be done by the use of a ball mill or a colloidal mill. In case oil or other finish is employed the same may be ground with the pigment or insoluble material.

The finishes containing the pigment or solid material may be applied to the yarn in any suitable manner. While we prefer to apply them to the yarn while it is in transit by means of rollers, rotating discs or the like which dip in a trough containing the finish, other means may be employed. Thus hanks of the yarn may be dipped in baths containing the finishes, or the finishes may be forced through the winding of a bobbin, cop or other package containing the yarn.

The finish containing the pigments or insoluble material may be applied to the artificial filaments or yarn immediately after their formation either within or outside of the spinning metier, or they may be applied in a winding operation prior to the knitting operation. If the finish containing the insoluble material or pigment is applied to yarn that is to be knitted, the same may be applied to the yarn immediately prior to its being fed to the knitting needles.

While very small amounts of pigment or insoluble material have a beneficial effect, we prefer to apply an amount equal to 0.2 to 2% based on the weight of the yarn, this being dispersed in an amount of oil or finish equal to between 5 and 15% of the weight of the yarn. Amounts in excess of these limits merely serve to increase the cost of operation and present the danger of fouling the guides, needles and other parts of the apparatus in which they come in contact because of the scraping off of the excess of finish and pigment.

The pigment or insoluble material added to the yarn may be removed from the fabric in any suitable manner such as by scouring, or in subsequent dyeing and finishing treatments. Often the removal of the pigments may be effected by chemical means; for example in case of calcium carbonate or barium phosphate, these may be removed by treatment with aqueous solutions of hydrochloric acid.

Yarn when treated by our invention has an increased coefficient of friction between the filaments. Moreover the frictional applied tension between the yarn and guides, knitting needles or other apparatus involved in textile operations is much more uniform. Because of this, knitted fabric may be made from yarn treated by our invention either by circular knitting or warp knitting machines, which fabrics are substantially free of distortions and pin-holes. This is of great importance in the making of hose particularly in circular knitting machines. Furthermore the so-treated yarn may be wound into packages, such as cones, bottle bobbins and the like which are very firm and which have less tendency to slip or collapse than packages previously made.

By way of illustration but without being

limited thereto, the following specific example is given.

*Example*

Yarn made by the twisting of a plurality of filaments of cellulose acetate has applied thereto a lubricant containing 9 parts of diethylene glycol and 1 part of titanium dioxide. This is done by passing the yarn over the upper surface of a slowly rotating roller, the roller dipping in a trough containing the finish. The rate of feed is so controlled that from 8 to 10% of diethylene glycol based on the weight of the yarn is applied.

The yarn so treated is then knitted in a circular knitting machine and a fabric is formed which is substantially free of stitch distortion and pin-holes.

It is to be understood that the foregoing details are given merely by way of illustration and that many variations may be made therein without departing from the spirit of this invention.

Having described our invention what we claim and desire to secure by Letters Patent is:

1. Method of forming knit fabrics comprising applying a finely divided solid to a yarn containing artificial filaments of organic derivatives of cellulose and then knitting the same whereby a knit fabric of substantially uniform loops is obtained.

2. Method of forming knit fabrics comprising applying a finely divided solid to a yarn containing artificial filaments of cellulose acetate and then knitting the same whereby a knit fabric of substantially uniform loops is obtained.

3. Method of forming knit fabrics comprising applying a conditioning liquid containing a finely divided pigment to yarn containing filaments of cellulose acetate and then circular knitting the same, whereby a knit fabric of substantially uniform loops is obtained.

In testimony whereof, we have hereunto subscribed our names.

CAMILLE DREYFUS.  
WILLIAM WHITEHEAD.

115

120

125

130